

## UNITED STATES PATENT OFFICE

1,980,889

## HEAT INSULATING MATERIAL

George Miller Thomson, Caledonia, Ontario,  
CanadaNo Drawing. Application December 21, 1931,  
Serial No. 582,509. In Canada December 17,  
1930

2 Claims. (Cl. 106—20)

The invention relates to heat insulating material of the type consisting of a pulverulent, granular or powdered mass of relatively mobile particles capable of being poured to form a heat insulating layer or partition. Many materials of this type are known, for example, ground wallboard, cork and the like.

A disadvantage of this type of insulating material is that, on account of its incoherent nature, it is compressible and therefore liable to settle or sag if subjected to shaking or vibration, thus increasing the density of the material and reducing its insulating efficiency, and also leaving an uninsulated space above the mass of material.

15 The present invention has for object to provide an improved material of the type described, in which the tendency to settle is greatly reduced, whereby, under normal conditions of use, the disadvantage above mentioned is substantially eliminated or, at least, reduced to negligible proportions.

With this end in view the invention consists in a heat insulating material of the kind described having small pieces of an exfoliated mineral substance of laminated form distributed throughout the mass.

The preferred mineral substance is vermiculite

treated with heat to cause its layers or laminations to exfoliate or partially separate, thus producing a light, flaky, non-inflammable material having air spaces between the layers. Pieces of this material of from about one-eighth to one-half inch 60 may conveniently be employed. According to a preferred form of the invention these pieces of exfoliated material are mixed as uniformly as possible with ground gypsum wallboard.

The greater the proportion of exfoliated material employed, the less will be insulating material be able to settle or sag when subjected to vibration. Good results have been obtained by mixing 40 to 50% of exfoliated vermiculite with 60 to 50% of ground gypsum wallboard. 70

What I claim is:

1. An article of manufacture consisting of a mass of ground gypsum wallboard having pieces of exfoliated vermiculite varying in size from one-eighth to one-half inch distributed throughout 75 the mass.
2. An article of manufacture consisting of a mixture of 40 to 50% by weight of exfoliated vermiculite and 60 to 50% of ground gypsum wallboard. 80

GEORGE MILLER THOMSON.

|    |     |
|----|-----|
| 30 | 85  |
| 35 | 90  |
| 40 | 95  |
| 45 | 100 |
| 50 | 105 |
| 55 | 110 |